

Nov. 18, 1947.

H. P. KIRCHNER

2,431,258

COATED ABRASIVE ARTICLE AND METHOD OF MANUFACTURING THE SAME

Filed Feb. 5, 1946.

*Fig. 1.*



*Fig. 2.*



*Fig. 3.*



*Inventor*

Henry P. Kirchner

by

*W. J. Foley*

Attorney

## UNITED STATES PATENT OFFICE

2,431,258

COATED ABRASIVE ARTICLE AND METHOD  
OF MANUFACTURING THE SAMEHenry P. Kirchner, Niagara Falls, N. Y., assignor  
to The Carborundum Company, Niagara Falls,  
N. Y., a corporation of Delaware

Application February 5, 1946, Serial No. 645,635

12 Claims. (Cl. 51—195)

**1**  
This invention relates to improved abrasive articles and to a method of manufacturing the same. It is particularly concerned with coated abrasive articles in which the backing comprises vulcanized fiber, and especially with discs made from such articles.

Abrasive discs of the kind with which this invention is particularly concerned have been described and claimed in a patent to Richard P. Carlton Re. 20,946. They are made by coating either vulcanized fiber alone or the cloth side of a combination of cloth and vulcanized fiber and very large numbers of such articles have been, and are being, made. They are used for a great variety of purposes, such as the removal of excess material from the welds on automobile bodies and for smoothing sheet material such as automobile fenders and refrigerator boxes.

The method by which these discs are commonly used is described and claimed in a number of patents, including a patent to Herbert R. Stratford No. 1,686,938. Their construction and method of use have been illustrated in the accompanying drawings, wherein:

Figure 1 is a side elevation of a disc made according to one modification of the present invention;

Figure 2 is a side elevation of a disc embodying a second modification of the invention; and

Figure 3 illustrates the manner in which the disc is employed.

As will be seen by reference to Figure 3, the discs are mounted on a rotatable shaft 13 by means of a nut 14 which screws into the end of the shaft and pulls the disc against a supporting pad 11 which is commonly made of felt or soft rubber. The pad is attached to the spindle 13 through a supporting element 12, which is commonly made of steel and is screwed tightly onto the outside of the spindle 13. As illustrated in the drawing, in use the discs are applied to the workpiece 15 at a slight angle so that only a portion of the periphery of the disc is in contact with the work at any particular instant. It will be apparent that the construction and method of use of the disc are such that a disc backing must be very tough and relatively stiff though flexible.

In order to make the disc fit snugly against the supporting pad 11 it is desirable that it should normally have a slight curvature with the abrasive coated side convex so that when the nut 14 is pulled into the spindle 13 the disc will be caused to hug the pad by reason of its springlike nature caused by the slight curvature. On the other hand, if the curvature of the disc is too great, the

**2**  
discs are very likely to crack when they are pulled up against the supporting pad by the nut 14. Likewise, if the disc has a curvature such that the abrasive side is concave, it will not lie snugly against the supporting pad and is very likely to catch against the work and tear.

It has been found by experience that a desirable curvature for the disc is such that the height of the cord of a disc 9 1/8 inches in diameter, which is a size which is very commonly used, shall lie within the range of about 1/4 inch to about 1 inch, and preferably shall be about 3/8 to 5/8 inch.

In order to obtain this desired degree of curvature it is common practice in the abrasive industry to cure the adhesive which is used for attaching the abrasive grains to webs of the backing material with the webs wound into rolls of such diameter that the curvature of the completed article falls within the desired range. After the material has been thus treated to set the adhesive the discs are stamped from the web material.

Although it is possible by this process to make discs which are initially of the desired curvature, a great deal of trouble is experienced by abrasive manufacturers by reason of the fact that vulcanized fiber is very susceptible to changes in atmospheric moisture content, particularly when one side of the material has been coated as is the case with the abrasive discs of this invention. It has been found, for example, that vulcanized fiber manufactured and sold by the Spaulding Fiber Company of Tonawanda, New York, under the trade-mark "Armit," which has been exposed to the air at 70° F. at 50% relative humidity contains 5.5% moisture whereas the same fiber exposed to air saturated with moisture contains 17.6% water. The fiber is therefore a relatively hygroscopic material and unfortunately when the moisture content of a fiber which has been coated on one side changes, the coated article curls. A reduction in the moisture content causes the fiber to curl with the coated side convex while an increase in moisture produces the opposite effect and causes the initially curved disc to become either flat or concave on the coated side. As has been pointed out above, either an extreme amount of curvature with the abrasive side convex or a reduction in curvature below the minimum limit of about 1/4 inch abrasive-convex makes the discs unsatisfactory.

It is accordingly an object of the present invention to provide a method of stabilizing abrasive discs having a backing comprising vulcanized fiber so that they are substantially unaffected

by changes in the atmospheric conditions to which they are exposed. Another object of the invention is to provide a method of treating abrasive discs to obtain a curvature in the desired direction and of a predetermined amount. Still another object of the invention is to provide abrasive discs which have a predetermined amount of curvature and which are substantially unaffected by changes in atmospheric moisture content whereby the discs retain the desired curvature.

I have found that the difficulties heretofore experienced with coated abrasive articles made on a backing comprising vulcanized fiber can be overcome and the objects of the invention can be accomplished by preliminarily drying the coated articles to obtain a desired curvature abrasive-convex, and then covering the vulcanized fiber with a sheet of material which is impermeable to moisture vapor. I accomplish this by any of several methods, one very satisfactory method being to dry the articles to such an extent that they assume an excessive amount of abrasive-convex curvature and then apply the water vapor-impermeable material by means of a water-soluble adhesive. One method which I have employed very successfully is to cut the abrasive discs from the web material, dry them until the moisture content is of the order of about 5-5.5%, as by heating in an oven for 2½ hours at 125° F., and then attaching a disc of paper-coated metal foil with the paper side against the vulcanized fiber. One such foil material which I have found to be satisfactory is made by the Reynolds Metal Company and identified as "Mat Silver #30 Unifoil." This material consists of a sheet of paper about .002 inch thick adhesively attached to an aluminum foil which is about .001 inch thick.

In carrying out the process I first coated the paper side of the "Unifoil" with ordinary mucilage which I allowed to dry and I then moistened the mucilage with water to make it tacky and pressed it against the back of a disc 9½" in diameter. I found that the small amount of water used to moisten the mucilage, which brought the moisture content of the disc to about 5.5-6%, was sufficient to make the disc assume a curvature such that the height of the cord formed by the curled disc was ¾ inch.

Referring now to the drawings:

In Figure 1 there is shown a side elevation of a disc having a backing 1 consisting of vulcanized fiber to one side of which a layer of abrasive grains 2 is attached by a bond 3. The other side of the fiber is provided with a layer of water vapor-impermeable foil 4 cemented to a paper layer 5 which is attached to the vulcanized fiber by an adhesive 6.

In Figure 2 the backing consists of a layer of vulcanized fiber 1 having attached to one surface a layer of cloth 7 by an adhesive 8 and to the other surface a water vapor-impermeable film 4 which is attached directly to the fiber by adhesive 6. As in Figure 1, the abrasive grains 2 are attached to the backing by a bond 3, in this instance the grains being directly applied to the cloth 7. The discs are provided with an arbor hole 9 for attaching to the spindle 13 in the manner illustrated in Figure 3. The amount of curvature of the discs shown in Figures 1 and 2 is indicated by the height *h* of the cord formed by the curved disc.

Although I have found the paper coated aluminum foil to be very satisfactory, I may use other metal foils such as copper and tin and I have also made discs which are stable to changes

in atmospheric moisture content by substituting for the metal foil other water vapor-impermeable materials such as a sheet of plasticized vinylidene chloride which is made by the Dow Chemical company and sold under the trade name "Saran," or by using a specially prepared paperlike product which is made by the Riegel Paper Corporation of New York city and sold under the designation "M. P. Heat Seal Laminated Amber Difane." Still another product of the Riegel Paper Corporation which has been found to be satisfactory for use in our invention is one sold under the designation "M. P. Heat Seal Pouch Stock." In applying these other materials I may either preliminarily cement them to a sheet of paper as was described with respect to the aluminum foil, or I may attach them directly to the disc by a suitable cement as shown in Figure 2 of the drawings.

In the latter case the disc is brought to the desired curvature before attaching the water vapor-impermeable film because it is necessary to use an adhesive made up with an organic solvent and such solvents do not materially affect the curvature of the fiber. For example, the "Saran" film may be attached by using a rubber cement which is substantially free from water. It is to be understood that the paper-foil film of Figure 1 may be used where the backing is a cloth-fiber combination, as shown in Figure 2, or that the film may be used without paper, as shown in Figure 2, where the backing consists only of vulcanized fiber.

Where I use a metal foil such as aluminum foil I have found that the foil is somewhat fragile and at times may be pricked or scratched, for example when it is put into contact with abrasive coated surfaces. To prevent such rupturing of the metal foil I find that it is sometimes desirable to apply a coat of lacquer over the metal foil. One such lacquer which I have found to be satisfactory has the following composition, the proportions being parts by weight:

|                       | Parts |
|-----------------------|-------|
| ½ sec. nitrocellulose | 16    |
| Ester gum             | 6     |
| Tricresyl phosphate   | 3     |
| Butyl alcohol         | 11    |
| Ethyl alcohol         | 7     |
| Butyl acetate         | 25    |
| Toluol                | 32    |

In applying such lacquer I first dilute the composition described above with an equal part of ethyl acetate and then spray this thinned lacquer over the metal foil. I have found that one coat is sufficient for my purpose and that a satisfactory weight is in the range of ¾ to 1½ grams of the lacquer solids per 100 square inches of foil. This corresponds to about 6 to 12 grams of the thinned lacquer per 100 square inches of surface since the thinned lacquer contains 87½% solvents.

It will be apparent that I may apply the lacquer either before or after the foil has been stuck to the disc. It will also be apparent that although I have described the application of the lacquer as a spray, it may be put on otherwise as by roll coating, in which case a lacquer may be employed of the composition given in the formula above and the thinning described for spraying is unnecessary.

As I have indicated, the backing may be either wholly vulcanized fiber or it may be a combination which includes vulcanized fiber such as a

combination of vulcanized fiber and cloth. I may also use other backing materials which include vulcanized fiber, such as a combination of cloth, paper and vulcanized fiber, as is described and claimed in my Patent No. 2,320,139 or I may even use conventional backings such as paper or cloth where the coated articles are to be employed for other purposes as in the manufacture of abrasive belts, sheets, cones or the like. Where fiber alone is employed I find it desirable to use a relatively thick material such as one about .030 inch thick. Where the fiber is combined with cloth, a very satisfactory article can be obtained by using a fiber which is .010 inch thick adhered to a drill cloth of the kind commonly used in the abrasive industry.

The abrasive grains may be attached to the backing by any suitable adhesive such as glue or a synthetic resin or by a combination of different adhesives. For example, they may be directly attached to the backing by a so-called "making coat" of glue and then a second or "sizing coat" of a synthetic resin such as a phenol-aldehyde condensation product may be applied over the abrasive grains and the glue making coat. Where a combination backing is used, the cloth backing may be cemented to the fiber by any suitable adhesive such as glue, a phenol-aldehyde resin, or a urea-aldehyde resin.

Although I have described my invention by reference to certain specific materials and methods, it is to be understood that the invention is not to be limited to the specific details described and shown in the drawings but rather is to be considered of the scope defined in the following claims.

I claim:

1. In a method of making an abrasive disc the steps which comprise bonding a layer of abrasive grains to a backing comprising vulcanized fiber, forming a disc from the abrasive coated backing, drying the article to such an extent that the abrasive coated side of the article is convex and the article has a radius of curvature which is smaller than that desired in the finished article, and attaching a sheet of paper adhesively joined to a film which is substantially impervious to water vapor on the vulcanized fiber on the side of the backing which is opposite the abrasive coating by an adhesive containing water whereby the water in the said adhesive penetrates the vulcanized fiber and causes the article to assume a predetermined curvature of greater radius than that of the dried article.

2. In a method of making an abrasive disc the steps which comprise bonding a layer of abrasive materials to a web of backing material comprising vulcanized fiber, cutting a disc from the abrasive coated web, drying the disc to such an extent that the abrasive coated side of the disc is convex, and adhesively attaching a preformed film which is substantially impervious to water vapor to the vulcanized fiber on the side of the backing which is opposite the abrasive coating.

3. In a method of making an abrasive disc the steps which comprise bonding a layer of abrasive materials to a web of backing material comprising vulcanized fiber, cutting a disc from the abrasive coated web, drying the disc to such an extent that the abrasive coated side of the disc is convex and the disc has a radius of curvature which is smaller than that desired in the finished article, and attaching a film which is substantially impervious to water vapor to the vulcanized fiber on the side of the backing which is oppo-

site the abrasive coating by an adhesive containing water whereby to increase the radius of curvature of the disc.

4. In a method of making an abrasive disc the steps which comprise bonding a layer of abrasive materials to a web of backing material comprising vulcanized fiber, cutting a disc from the abrasive coated web, drying the disc to such an extent that the abrasive coated side of the disc

10 is convex and the disc has a radius of curvature which is smaller than that desired in the finished article, and attaching a sheet of paper adhesively joined to a sheet of metal foil to the vulcanized fiber on the side of the backing which is opposite the abrasive coating by a water-soluble adhesive, the amount of water in the adhesive being such as to cause the finished disc to assume a curvature such that the height of a cord formed by a disc about 9 inches in diameter is within 20 the range of about  $\frac{1}{4}$  to 1 inch.

5. In a method of making an abrasive disc the steps which comprise bonding a layer of abrasive materials to a web of backing material comprising vulcanized fiber, cutting a disc from the

25 abrasive coated web, drying the disc to such an extent that the abrasive coated side of the disc is convex and the disc has a radius of curvature which is smaller than that desired in the finished article, and attaching a sheet of paper adhesively

30 joined to a sheet of aluminum foil to the vulcanized fiber on the side of the backing which is opposite the abrasive coating by a water-soluble adhesive, the amount of water in the adhesive being such as to cause the finished disc to assume a curvature such that the height of a cord formed by a disc about 9 inches in diameter is within 35 the range of about  $\frac{1}{4}$  to 1 inch.

6. An abrasive disc comprising a backing comprising vulcanized fiber, a layer of abrasive grains bonded to one side of the backing, and a film which is substantially impervious to water vapor

40 adhesively attached to the vulcanized fiber on the side of the backing which is opposite the abrasive coating, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in 45 atmospheric moisture conditions.

7. An abrasive disc comprising a backing comprising vulcanized fiber, a layer of abrasive grains bonded to one side of the backing, and a layer of paper adhesively joined to a film which is sub-

60 stantially impervious to water vapor attached to the vulcanized fiber on the side of the backing which is opposite the abrasive coating by a water-soluble adhesive, the moisture content of the vulcanized fiber being such that the disc has a

65 curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in 70 atmospheric moisture conditions.

8. An abrasive disc comprising a backing com-

prising vulcanized fiber, a layer of abrasive grains bonded to one side of the backing, and a layer of paper adhesively joined to a sheet of metal foil attached to the vulcanized fiber on the side of the backing which is opposite the abrasive coating by a water-soluble adhesive, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in atmospheric moisture conditions.

9. An abrasive disc comprising a backing comprising vulcanized fiber, a layer of abrasive grains bonded to one side of the backing, and a layer of paper adhesive joined to a sheet of aluminum foil attached to the vulcanized fiber on the side of the backing which is opposite the abrasive coating by a water-soluble adhesive, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in atmospheric moisture conditions.

10. An abrasive disc comprising a backing comprising vulcanized fiber and cloth, a layer of abrasive grains bonded to the cloth, and a film which is substantially impervious to water vapor adhesively attached to the other side of the vulcanized fiber, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in atmospheric moisture conditions.

10  
15

20

25

30

35

40

45

50

11. An abrasive disc comprising a backing consisting of vulcanized fiber, a layer of abrasive grains bonded to one side of the fiber, and a film which is substantially impervious to water vapor adhesively attached to the other side of the vulcanized fiber, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in atmospheric moisture conditions.

12. An abrasive disc comprising a backing comprising vulcanized fiber, a layer of abrasive grains bonded to one side of the backing, a layer of paper adhesively joined to a sheet of aluminum foil attached to the vulcanized fiber on the side of the backing which is opposite the abrasive coating by a water-soluble adhesive, and a coat of lacquer on the exposed side of the aluminum foil, the moisture content of the vulcanized fiber being such that the disc has a curvature in such direction that the abrasive surface is convex and of such an amount that the height of a chord formed by a disc about 9 inches in diameter is within the range of about  $\frac{1}{4}$  to 1 inch, the vulcanized fiber being so sealed in by the bond for the abrasive grain on the one side and the film on the back that the curvature of the disc remains within the designated range even when the disc is exposed to wide variations in atmospheric moisture conditions.

HENRY P. KIRCHNER.

## REFERENCES CITED

The following references are of record in the file of this patent:

## UNITED STATES PATENTS

| Number    | Name         | Date          |
|-----------|--------------|---------------|
| 2,269,661 | Gurwick      | Jan. 13, 1942 |
| 2,190,479 | Moore        | Feb. 13, 1940 |
| 1,759,168 | Okie         | May 20, 1930  |
| 2,152,392 | Tone         | Mar. 28, 1939 |
| 1,966,473 | Woodell      | July 17, 1934 |
| 2,085,211 | Budds et al. | June 29, 1937 |